

## UNITED STATES PATENT OFFICE

KENNETH B. CHURCH, OF NORWICH, CONNECTICUT, ASSIGNOR TO THE ASPINOOK COMPANY, OF JEWETT CITY, CONNECTICUT, A CORPORATION OF CONNECTICUT

## METHOD OF WATERPROOFING FABRICS

No Drawing.

Application filed April 17, 1926. Serial No. 102,808.

This invention relates to a method or process of treating fabric wherein a colored or printed product is provided which is waterproofed and otherwise treated to give both 5 an inside and outside finish.

The object of the invention is to treat a piece of cloth so as to present an inside and an outside finish while at the same time causing the cloth to be waterproof.

10 A further object of the invention is to provide a process or method of treating cloth wherein a waterproof product will be produced which will be substantially as flexible as the cloth before its treatment.

15 A still further object, more specifically, is to provide a process or method of treating cloth whereby a duplex effect is produced for causing the cloth to present a different appearance on each side.

20 In carrying out the objects of the invention, a piece of cloth of any desired size may be used, as for instance, a piece of ordinary twill cloth which is first dyed or printed by the regular process of dyeing or printing or 25 in any preferred manner. This cloth is then given one coat of pyroxylin on one side after which it is subjected to a finishing action, as for instance, by a Schreiner roll which gives the desired impression upon the reverse face.

30 The cloth is then returned to the coating machine and given two more coats of pyroxylin on the coated surface. It is evident, however, that more or less coats could be provided without departing from the spirit of the invention 35 and also the finishing may be done as described or after all the coats have been applied.

By applying the coating on one side the goods are reversible and thereby adapted for 40 many uses, as for instance, raincoats, where the coated side may be exposed to the weather and the machine finished side will take the place of the lining and have the appearance of the same. The pyroxylin solution may be 45 colored or clear as desired. By applying a coating of this solution on one side of a piece of cloth and providing an embossed lining finish on the other, a duplex effect on one fabric is the result.

50 Preferably, the pyroxylin coating is a solu-

tion of nitrocellulose, solvent, plasticizers and gums. This coating is preferably applied in the regular type coating machine or in any other convenient manner. On the uncoated side, the desired effect is produced by running 55 the cloth through a pressure calender under a hot engraved steel roll on which lines or other suitable designs have been engraved. This action may take place before the cloth is coated or after any coating. The finished 60 product is very pliable and pleasing in appearance.

What I claim is:

The process of treating a piece of cloth to produce a duplex effect thereon consisting 65 in applying coloring matter to the cloth, giving the cloth a preliminary coating of pyroxylin on one surface, subjecting the other surface to an impression roller under pressure until a desired impression has been formed on 70 said other surface, and finally applying a second coating of pyroxylin over the first coating.

KENNETH B. CHURCH.

75

80

85

90

95

100